

# UNITED STATES PATENT OFFICE.

MICHAEL ILJINSKY, OF UERDINGEN-ON-THE-RHINE, GERMANY, ASSIGNOR TO MESSRS. WEDEKIND & CO., M. B. H., OF UERDINGEN-ON-THE-RHINE, GERMANY.

## PROCESS FOR DYEING WITH DYESTUFFS INSOLUBLE IN WATER OR WATER-INSOLUBLE LEUCO COMPOUNDS OF DYESTUFFS.

1,199,273.

Specification of Letters Patent. Patented Sept. 26, 1916.

No Drawing.

Application filed December 10, 1912. Serial No. 735,930.

To all whom it may concern:

Be it known that I, MICHAEL ILJINSKY, chemist, subject of the Czar of Russia, residing at Uerdingen-on-the-Rhine, Germany, have invented a new and useful Process for Dyeing with Dyestuffs Insoluble in Water or Water-Insoluble Leuco Compounds of Dyestuffs; and I do hereby declare the following to be a full, clear, and exact description of the same.

Experimental investigations have led to the extremely surprising and technically important result that many dyeing compounds insoluble in water, such as vat dye-stuffs, water-insoluble leuco-metal salts of the vat dye-stuffs (leuco-salts of magnesium, zinc, alumina, tin, etc.), and mordant dye-stuffs such as alizarin or others, are in neutral, acid or alkaline aqueous suspension capable of acting readily even cold upon unmordanted or previously mordanted vegetable or animal fibrous materials and in this way to form with the fiber a kind of loose or unstable compound which possesses, however, sufficient stability to be thereafter in one way or another transformed into stable and fast dyeings. It is very surprising that in this way uniform and well-penetrated dyeings can be obtained.

The technical advantages of this method are manifold. Since the dye-baths can be kept very concentrated, large and therefore expensive dye-vats become unnecessary; the costly extended boiling of large quantities of liquid in mordant dyeing is likewise suppressed, as well as the movement of the goods treated therein. Since the absorption of the dye-stuffs, if certain conditions are observed, takes place so well as to be without residue, the vat dyer is able to carry out the dyeing with accurately measured quantities of dyestuff. The troublesome and time-wasting restoration of the vat to the desired content of dye-stuff becomes unnecessary. In particular with mixed tints of two or more dye-stuffs which in leuco form act upon the fibrous material in the vat with differing rapidity, the technical advantage of the method becomes clear. A further advantage is due to the circumstance that the equalization of the dyestuffs

takes place upon the formation of the first unstable compound. The dyer is, therefore, relieved of the trouble of the equalization in carrying out the second part of the dyeing process, the transformation of the unstable dye-stuff compound into the stable form, that is to say in the actual dyeing, so that this second operation can be undertaken in closed mechanical apparatus. From all these advantages there results a considerable cheapening of the dyeing.

The more concentrated the dye-baths are kept, the quicker and more thorough is the absorption of the dye-stuff suspended in the bath. The greatest affinity for the dye-stuffs suspended in water is shown by silk fibers, wool fibers coming next. In the case of cotton, it is necessary to adhere to considerably more concentrated dye-baths, if it is desired to obtain a thorough absorption of the dyestuff. If the bath is too concentrated, the dyeings turn out slightly uneven. However, sufficient equalization can be finally obtained by padding the goods in the cold for a longer time.

The formation of the first unstable compounds of the dyestuffs with the fiber takes place with vat dyestuffs in the same way as with mordant dyestuffs insoluble in water; during the second process, the transformation of the unstable into the stable dyeing proper, it is necessary to resort to various processes according to the nature of the dyestuffs.

In the case of vat dye-stuffs, the unstable dyeing, which is sufficiently resistant to cold and warm water, but not to soap, may be successfully transformed into a fast dyeing by vatting the unstable compound upon the fibrous material and then oxidizing it in the air. It is remarkable, that with the correct method of working no quantity of the dyestuffs worth mentioning is in this way dissolved from the fiber. In the German patent specification 177952 (class 8<sup>m</sup>), there is described a process according to which the dyestuff thickened with glue, rubber, etc., is spread upon the cotton material, and the material so prepared is then treated with an alkaline reducing solution. But that process is only patented for indan-

threne dyestuffs (it is expressly mentioned in the description that no useful results are obtained with indigo), whereas the method of the present invention is capable of general application. Further, the two methods have nothing in common for the reason that it was not to be foreseen that the unreduced vat dyestuffs would also be able to act upon the fibers without adhesives, in the insoluble form and from aqueous suspension, and that in spite of the absence of adhesive, these additions of dye-stuff are for the greater part not again dissolved by the alkaline reducing solution. In the process of the present invention, the insoluble dyeing compounds are free from adhesives, thickening or sulfur.

In the case of mordant dyestuffs insoluble in water, it is sufficient to steam or to heat under water the water-resisting unstable dye-stuff compounds. The methods of working will be explained by the following examples:—

#### A. VAT DYESTUFFS.

25

##### *First operation—Unstable combination of the dyestuff.*

Example 1: 10 kilograms of cotton, dry or moistened, are padded at ordinary temperature in 40 liters of neutral or feebly alkaline indigo suspension, containing 200 grams of indigo. The absorption of the dyestuff is completed in a few minutes. The padding is continued a little longer, whereby the equalization is very considerably promoted.

Example 2: 10 kilograms of cotton are padded as in Example 1 in 40 liters of a neutral or feebly alkaline suspension containing 200 grams of algol-orange with 100 grams of algol-blue.

Example 3: 10 kilograms of cotton are padded as in Example 1 in 50 liters of a neutral or feebly alkaline suspension containing 150 grams of indanthrene and 150 grams of thioindigo-red.

Example 4: 10 kilograms of wool, dry or moistened, are padded as in Example 1 with 50 liters of a neutral or feebly acid suspension of algol-yellow, containing 200 grams of dyestuff.

Example 5: 10 kilograms of silk in a moist condition are stirred at the ordinary temperature as for acid dyeing in 200 liters of a neutral or feebly acid suspension, containing 300 grams of algol-orange. The absorption of the dyestuff is completed in a few minutes.

##### *Second operation.*

The vatting upon the fiber is in all cases carried out in such a manner that after the absorption of the dyestuff in the first operation the wrung-out goods are placed in an

alkaline hydrosulfite solution, which is preferably mixed with common salt or sulfate. The quantity of alkali and of hydrosulfite must be determined according to the nature of the dyestuff, and for example in the case of indanthrene it will be much greater than with indigo or algol dyes. The total quantity of liquid need be only large enough to cover evenly the goods in an unpressed condition. In the preferred manner of working, which in any special case can easily be determined, the dyestuff may with success be reduced upon the fiber in such a way, that no quantity worth mentioning is dissolved from the fiber. After the reduction is completed, the goods are wrung, hung out, wound and soaped.

#### B. MORDANT DYESTUFFS.

##### *First operation—Formation of the unstable lake.*

Example 6: 10 kilograms of cotton mordanted with alumina as usual for Turkey-red ready for dyeing, are padded at ordinary temperature with 50 liters of a suspension, containing 200 grams of alizarin with or without addition of acetate of lime and Turkey-red oil. The absorption of the dyestuff is completed in a few minutes.

Example 7: 10 kilograms of cotton mordanted for dyeing as usual for Turkey-red, are padded as in Example 6 with 50 liters of a suspension containing 100 grams of alizarin and 100 grams of anthrapurpurin.

Example 8: 10 kilograms of wool, chrome mordanted as usual are stirred at the ordinary temperature as for acid dyeing, in 60 liters of a neutral or feebly acid suspension, containing 200 grams of flavopurpurin with or without addition of acetate of lime and Turkey-red oil. The absorption of the dye is effected in a few minutes.

Example 9: 10 kilograms of yarn oil-mordanted as usual for old-red or new-red are well moistened. The wrung-out goods (weight about 20 kilograms) are thoroughly kneaded for about ten minutes in the following bath:—45 kilograms of water, 1800 grams of crystallized aluminium sulfate, 3500 cubic centimeters of acetate of lime of 17 degrees Baumé, and 100 grams of a 20 per cent. alizarin-paste.

Example 10: 10 kilograms of yarn oil-mordanted and moistened as in Example 9 are thoroughly kneaded for ten minutes in the following bath:—47 kilograms of water, 1400 cubic centimeters of ferrous sulfate solution 1:10, 180 grams of crystallized sodium acetate, and 100 grams of a 20 per cent. alizarin-paste.

Example 11: (Single-bath process). 10 kilograms of unoiled and unmordanted yarn are wetted and the wrung-out goods weighing about 20 kilograms, are then thoroughly

80

90

95

100

105

110

115

120

125

130

kneaded for about ten minutes in a bath of: 27 kilograms of water, 600 grams of crystallized sodium acetate, 1500 cubic centimeters of acetate of lime of 17 degrees Baumé, 1800 5 cubic centimeters of acetic acid of 6 degrees Baumé, 200 grams of 50 per cent. Turkey-red oil F, 1000 grams of a 20 per cent. alizarin-paste.

10 *Second operation—The production of the lake.*

The formation of the lake begins to take place already at cold after the action of the alizarin dyestuff upon the mordanted fiber. By the progressive deeper dyeing of the 15 goods one can very clearly trace the progress of the formation of the lake. However days are necessary in order to effect the formation of the lake at ordinary temperature in any way completely. If the goods are not 20 oil-mordanted, it is important after the boiling and before the production of the lake to dry the goods for some time at 60 to 70 degrees centigrade. Upon warming in the 25 moist state, the formation of the lake takes place almost instantaneously, which operation however is preferably not effected at once after the kneading but after allowing to stand for some time. A quarter to half an hour boiling under water suffices to produce the lake. A still more permanent lake 30 is formed, if the wrung-out goods after the first operation are steamed under a pressure of one to one and a half atmospheres. Since 35 neither water or steam dissolves the lake which is in an unstable state combined with the fibers of the latter, the goods can be brought into the boiling or steaming apparatus for boiling under water with addition of common salt or sulfate if so desired or 40 for steaming simply in heaps laid upon one another. Any movement, stirring or similar manipulation is unnecessary, and the quantity of water has no influence. On the other hand its hardness must be taken into 45 consideration. The brightening of the dyed goods is effected in the usual way.

C. COMBINATION OF VAT AND MORDANT DYESTUFFS.

50 Example 12: 10 kilograms of cotton mordanted with alumina ready for dyeing as usual for Turkey-red are padded at normal temperature with 50 liters of a suspension containing 150 grams of algol-yellow with 55 or without addition of acetate of lime and Turkey-red oil. The absorption of the alizarin as well as of the algol-yellow is completed in a few minutes.

Example 13: 10 kilograms of wool chrome 60 mordanted as usual are padded at ordinary temperature in 60 liters of a feebly acidulated suspension containing 200 grams of alizarin and 50 grams of algol-yellow. The absorption of the dyestuffs is completed in a few minutes.

*Second operation.*

The wrung-out dyed goods are first either warmed under water or steamed for the purpose of producing the alizarin lake. In order to fix the vat dyestuff, which is not dissolved either upon steaming or by boiling of the dyestuff under water, it must subsequently be vatted. The alizarin lake once formed does not suffer thereby; provided the vatting is done in a careful manner. After winding and soaping there are obtained in this way thoroughly fast mixed tints.

10 D. MAGNESIUM LEUCO COMPOUNDS OF VAT 80 DYESTUFFS.

In dyeing with vat dyestuffs as hitherto practised, the dyestuff is always converted into the soluble leuco compound usually by means of a reducing agent in presence of 85 strong alkali such as soda-lye, ammonia or lime. This applies also for example in the case of zinc-lime and ferrous sulfate-lime indigo-vats, in which the reducing agent is insoluble, but the resulting indigo-white is 90 converted into the soluble form by means of calcium hydroxid. As has been proved by investigations, vat dyestuffs such as indigo and its derivatives, dyestuffs of the thio-indigo series, and algol-dyes are in the presence of magnesium hydroxid capable of acting evenly upon the fibers in an aqueous suspension of their magnesium leuco compounds which are only slightly soluble in 95 water. It is remarkable that in this case the absorption of the dyestuff is effected much more completely than by the use of soluble alkali leuco compounds, in which case as is known it is always necessary to work in the vat with an excess of dyestuff. This is another example of the surprising phenomenon that dyestuffs insoluble in water are enabled to act upon the fibers at ordinary temperature.

The advantages of the magnesia vats are manifold. Since magnesium hydroxid has hardly any alkaline reaction, the magnesia vats are specially suitable for wool and silk, which as is known do not stand alkali well. This opens up the possibility of 110 dyeing wool and silk with vat dyestuffs in many cases in which the use of vat methods has hitherto been scarcely feasible. Since the combination of the magnesium leuco compounds of the vat dyestuffs with the 115 fibers is at first only loose, the dyestuff can be well equalized by a slight movement or padding of the goods or by mechanical circulation of the bath, before the more fixed intermediate combination of the dyestuff is 120 brought about. It is also important that for the concentrated baths characterizing the process, the dimensions of the vats are naturally small. A more important point is that magnesia vats oxidize by the influence of 130

air far more slowly than soda or lime baths, which circumstance allows a more convenient and more tractable working.

Example 14: 200 grams of algol-yellow in the form of paste are added to 50 liters of water containing 400 grams of magnesium hydroxid and 600 grams of hydrosulfite. After a short time the formation of the orange-red suspension of the magnesium leuco compound is completed. 10 kilograms of cotton are then entered. The action of the suspended magnesium leuco compound proceeds in a short time and can be accelerated by moving or padding the goods or by circulating the liquor. The progressive orange dyeing of the goods together with the decoloration of the suspension indicate the progress of the operation. After the absorption of the dyestuff is completed, the goods are wrung, hung out, wound, acidulated and soaped. The evenness and the fastness of the dyeing leave nothing to be desired.

Example 15: 200 grams of indigo in paste are stirred into 50 liters of water containing 400 grams of magnésium hydroxid and 600 grams of hydrosulfite. After a short time the formation of a light green suspension of magnesium-leuco compounds of indigo is completed. 10 kilograms of wool are entered and treated as in Example 14. The evenness and fastness of the dyeing are excellent.

Example 16: 200 grams of thioindigo-red in paste are added to 50 liters of water, containing 400 grams of magnesium hydroxid and 600 grams of hydrosulfite. As soon as the formation of the yellow magnesia leuco compound is completed, 10 kilograms of silk are entered and treated as in Example 14. The evenness and fastness of the dyeing are remarkable.

Example 17: 10 kilograms of cotton are padded in a suspension consisting of 40 liters of water and 150 grams of thioindigo-red, 50 grams of algol-yellow and 400 grams of magnesium hydroxid until the absorption of the dyestuff is completed. 600 grams of hydrosulfite dissolved in 10 liters of water are then added. After the reduction upon the fiber is completed, the goods are wrung, hung out, acidulated and soaped. It is also possible to proceed by first wringing out the goods which have been padded with algol-yellow in the presence of magnesium hydroxid and then introducing them into the necessary quantity of hydrosulfite solution, because in the padding not only the dyestuff but also the magnesium hydroxid is absorbed and fixed by the fiber. The dyes turn out even and of good fastness.

The concentration of the liquors, the proportions of the mixture of magnesium hydroxid and hydrosulfite and also the temperature may be varied within wide limits.

Instead of vatting the vat dyestuffs with hydrosulfite only in the presence of magnesium hydroxid, it is also possible to proceed by effecting the vatting with hydrosulfite in an alkaline solution (soda or lime) with or without addition of magnesium hydroxid, after which sufficient quantities of a metal salt such as magnesium chlorid, aluminium sulfate, zinc sulfate, stannous chlorid, stannic chlorid, etc., are added, and the action of the dyestuff from the suspension of the corresponding insoluble metal leuco compound is accomplished. In this way the alkalinity of the vat may be reduced as desired, even indeed so far as to be able to work with a vat showing an acid reaction upon litmus.

In dyeing with magnesium and other metal leuco compounds of the vat dyestuffs there may also be employed for the purpose of producing darker tints vat-additions of greater strength, in which case the quantities of dyestuff consumed must be restored for the next operation. In this way it is possible to produce upon wool for example in one operation extremely powerful dyeings of very good fastness.

In general feeble dyeings are produced by diluted baths, strong ones by concentrated baths. Apart from the concentration of the bath the temperature during dyeing is also of importance. Cotton absorbs better from cold baths, wool from warm ones and silk from tepid ones. It is therefore practicable in the case of mixed textile fibers to produce any desired effects, by dyeing either all the fibers evenly in tepid baths or only one fiber as preferred.

Further experiments have shown that animal fibers (wool or silk) may be caused to absorb vat dyestuffs in a quantitative manner from quite diluted baths, if the reaction is assisted by warming. In this way vat dyestuffs may be fixed simultaneously, which otherwise could only with difficulty be dyed in the vat beside one another on account of their varying affinity for vat dyestuffs. New effects may be obtained by dyeing vat dyestuffs combined with acid or mordant dyestuffs in one bath. Also in this case quite definite proportions of quantities of the components may be determined from the foregoing. If one has to deal exclusively with vat dyestuffs, one may proceed further in order to convert the unstable compound into the dyeing proper, as has been done above in the second operation. In combined dyeings by vat dyestuffs with mordant dyestuffs, the goods are subsequently submitted to vatting, then hung out, wound and soaped.

The vat dyestuff combined in an unstable condition with the fiber is thereupon converted into the stable compound proper. The metal lakes of the mordant dyestuffs already formed upon the fibrous material

remain unaffected by alkaline vats provided their alkalinity, concentration and temperature do not exceed certain limits. After vatting the goods are hung out, wound and soaped.

Example 18: 200 grams of indigo and 200 grams of algol-yellow are suspended in 200 liters of water; the liquid is acidulated with acetic acid and 10 kilograms of moistened 10 woolen yarn are entered. The temperature is gradually raised to 60 degrees centigrade, with frequent movement of the goods. After the goods have been allowed to cool, the quantity of dyestuff taken up is fixed 15 upon the fiber in a feebly alkaline hydro-sulfite solution or in a magnesium hydroxid-hydrosulfite vat. Afterward the goods are hung out, wound and soaped.

Example 19: One proceeds as given in 20 Example 18, but in place of woolen yarn the same quantity of Chappe-silk is used.

Example 20: 200 grams of indigo and 200 grams of thioindigo-red to 10 kilograms of 25 woolen yarn. Dyeing is effected as in Example 18.

Example 21: Dyed as in Example 20, but instead of woolen yarn, the same quantity of Chappe-silk is treated.

Example 22: 200 grams of alizarin and 30 200 grams of indigo; 10 kilograms of silk prepared for Turkey-red are dyed as prescribed in Example 18.

Example 23: 200 grams of alizarin and 200 grams of indigo; 10 kilograms of chrome 35 mordanted woolen yarn are dyed as stated in Example 18.

Example 24: 200 grams of quinoline-yellow and 200 grams of indigo; 10 kilograms of Chappe-silk are dyed as in Example 18 40 described.

Example 25: 200 grams of algol-yellow, 10 kilograms of woolen yarn are treated as in Example 18.

The term "dyeing compounds" used in 45 the above description and in the claims covers vat dye-stuffs, leuco-metal salts of the vat dye-stuffs and mordant dye-stuffs of the alizarin series.

Having thus described my invention, what 50 I claim as new and desire to secure by Letters Patent is:

1. A process for dyeing with dyeing compounds insoluble in water, said process comprising bringing the goods to be dyed into

contact with an aqueous suspension of dye- 55 ing compounds insoluble in water and free from sulfur and thickening; and then converting the resulting unstable dyestuff compounds into stable dyeings proper.

2. A process for dyeing with dyeing compounds insoluble in water, said process comprising bringing the goods to be dyed into contact with an aqueous suspension of dye- 60 ing compounds insoluble in water and free from sulfur; and then converting the re- 65 sulting unstable dyestuff compounds into stable dyeings proper.

3. A process for dyeing with dyeing compounds insoluble in water, said process comprising bringing the goods to be dyed into 70 contact with an aqueous suspension of dyeing compounds insoluble in water and free from thickening; and then converting the resulting unstable dyestuff compounds into stable dyeings proper. 75

4. A process for dyeing with vat dye- 80 stuffs insoluble in water comprising first bringing the goods into contact with an aqueous suspension of the dyeing compounds insoluble in water, and then converting the resulting unstable dyestuff compounds into stable dyeings proper by subsequent vatting upon the fiber and oxidizing the leuco compounds formed.

5. A process for dyeing with dyeing com- 85 pounds insoluble in water, said process comprising bringing the goods to be dyed into contact with a cold concentrated aqueous suspension of dyeing compounds insoluble in water and free from thickening; and then 90 converting the resulting unstable dyestuff compounds into stable dyeings proper.

6. A process for dyeing with vat dyestuffs insoluble in water comprising first bringing goods into contact with an aqueous suspen- 95 sion of the dyeing compounds insoluble in water, and then converting the resulting unstable dyestuff compounds into stable dye- 100 ings proper by subsequent vatting upon the fiber and oxidizing the compounds formed.

In testimony whereof, I have signed my name to this specification in the presence of two subscribing witnesses.

MICHAEL ILJINSKY.

Witnesses:

FRANZ RANENSTEIN,  
HENRY QUADFLIEG.